

L. B. LINDEMUTH.

HOT TOP.

APPLICATION FILED OCT. 13, 1919.

1,332,906.

Patented Mar. 9, 1920.

Fig. 1.



Fig. 2.

Fig. 3.

Fig. 4.

Fig. 5.



Inventor

Lewis B. Lindemuth

by Henry Orth Jr.

atty

# UNITED STATES PATENT OFFICE.

LEWIS B. LINDEMUTH, OF NEW YORK, N. Y.

## HOT-TOP.

1,332,906.

Specification of Letters Patent. Patented Mar. 9, 1920.

Application filed October 13, 1919. Serial No. 330,275.

To all whom it may concern:

Be it known that I, LEWIS B. LINDEMUTH, a citizen of the United States, residing at New York city, in the State of New York, United States of America, have invented certain new and useful Improvements in Hot-Tops; and I do hereby declare the following to be a full, clear, and exact description of the invention, such as will enable others skilled in the art to which it appertains to make and use the same, reference being had to the accompanying drawings, and to letters or figures of reference marked thereon, which form a part of this specification.

My invention relates to sink-heads, feeders, or so-called "hot tops" used in the casting of ingots and other heavy castings.

I have invented a hot-top made of sheet metal, and the present invention is an improvement on metal hot-tops in which, preferably, that portion of the top which is positioned below the top of the mold is preferably provided with a continuous peripheral depression, fold, or the like, that decreases the cross-section of the ingot or casting, thereby forming a groove therein.

This groove may be positioned at any desired point of the casting within the limits of operation of the hot-top, by raising or lowering the top with respect to the mold. The positioning can readily be accomplished, as the sheet metal hot-top is frictionally held in the top of the mold. The hot-top becomes welded to the ingot or casting, and when the ingot is removed from the mold it presents, preferably, a continuous peripheral groove or nick formed by the indentation in the hot-top, so that the ingot can be readily cropped, the nick or groove determining the breaking point of the crop end from the body of the ingot. This can readily be done under a power hammer.

Inasmuch as the hot-top is frictionally held in the top of the ingot mold, it may be raised or lowered at will, to suit any condition desired, so that the nick will be located in the ingot or casting as required.

Referring to the drawings, in which like parts are similarly designated—

Figure 1 is a cross section showing the hot-top applied to an ingot mold.

Figs. 2-5 are enlarged cross-sectional views illustrating different shapes for the fold, groove, crimp or the like in the hot-top.

Referring to Fig. 1, the hot-top or sink-head 5 is composed of sheet metal, the thickness being exaggerated in the drawings for the sake of clearness. The sheet metal of the hot-top 5 is preferably shaped around a suitable form to fit the desired size of ingot mold 1. The edges of the sheet metal overlap and are secured together by means of a few rivets 12, by spot-welding, or any approved form of connection.

Near the bottom of the hot-top 5 is formed, a preferably continuous crimp, *a*, shown in this particular figure as V-shaped in cross-section. The crimp is inwardly directed and reduces the cross-section of the ingot at the point where the crimp is located.

The crimp may be made to diminish the cross section of the mold and casting any desired extent, but under ordinary circumstances it is dimensioned about 10% of the internal diameter of the mold, so that there will be a reduction of about 20% of the cross sectional area. It is preferable, however, to maintain the reduction of area as low as possible consistent with the breaking properties of the particular metal. For example, in order to easily crop an ingot of high carbon steel, the depth of notch should be greater than for an ingot of high speed steel, and similarly low carbon steel ingots will have to be more deeply notched than high carbon steels, so that the crimps *a* will be dimensioned to conform to the particular composition of metals to be cast.

Surrounding the sink head or hot-top 5 is a packing retainer or box 6 having a bottom flange 7 that rests on the top of the mold 1, leaving an annular space 8 between the edge of said flange 7 and the hot-top 5. The space between the box 6 and top 5 is filled with loose dry sand, or other non-conductor of heat. If desired, a packing 13 of clay, asbestos rope or equivalent may be placed in the annular space 8 to prevent any sand from passing into the mold between the contacting surfaces of the hot-top 5 and the mold 1.

The hot-top being of sheet metal and supported by frictional contact with the interior walls of the mold is, after casting, free to slide down into the mold upon the cooling of the casting, while the metal in the hot-top 5 above the top of the mold 1 is kept hot by the heat insulating material 11.

The notch in the casting may easily be

formed at a higher or lower level by inserting the hot-top 5 to a greater or less extent into the top of the mold.

The hot-top becomes welded to the casting 5 and is used but once. The part above the crimp and broken off with the crop end goes into the scrap, while the lower part adhering to the body of the ingot will disappear in the subsequent heat treatments, 10 or other usual manipulations of ingots and castings.

The material of which the hot-top is made is preferably of the same composition as the metal cast, so as not to alter the composition 15 of the crop ends used as scrap metal.

The hot top, though thin and of the same composition as the metal poured, does not melt because the material of the hot top is cold, and the moment that the molten metal 20 comes into contact with it a thin layer of the molten metal solidifies to the surface of the hot top. This quick chilling of a thin section of the surface of the ingot is sufficient to keep the hot top from melting.

25 In Fig. 1 I have shown the hot-top applied to a very small ingot, say about four inches in diameter, the metal is about 22 gage sheet steel, or about 0.0312 inches thick, the depth of the crimp about three-eighths 30 of an inch, and the angle included between the sides of the crimp is about  $60^\circ$ . The diameter of the container 6 is about eight inches with about one-quarter of an inch thickness of its walls.

35 In Fig. 2 I have shown another form of crimp  $a'$  where the sides of V-shaped crimp Fig. 1, are brought close together.

In Fig. 3 the crimp  $a^2$  is semicircular in cross section.

40 In Fig. 4 the crimp  $a^3$  is rectangular in cross section, having substantially parallel walls  $b$  connected by a straight end wall  $c$ .

In Fig. 5 the crimp  $a^4$  is formed by combining the structures shown in Figs. 1 and 4, 45 having substantially parallel walls  $b$  connected by a V-shaped end wall  $d$ .

50 My invention is not limited to the particular shape of the crimp, as any shape that can be easily made may be used, however, experience shows that the simple V-shaped crimp can be very easily rolled into the sheet metal before forming the hot-top around a suitable form.

Nor is the invention limited to the formation of a continuous groove in the casting. For example, for polygonal ingots the crimps can be located at alternate sides, or on opposite sides, and especially would this be effective in castings whose cross sections 55 are oblong, the crimps being arranged at the long sides of the cross section, so that the

ingot will be indented only on its larger surfaces.

I claim—

1. The combination with a casting, of a 65 hot-top having a groove-forming crimp, said hot-top in welded connection with the casting.

2. A sheet metal hot-top having a crimp therein for forming a groove in a casting. 70

3. A hot-top, comprising a sheet of metal having a crimp therein and having its edges secured together, the crimp operating to diminish the internal cross section and thereby form a groove in a casting. 75

4. A sheet metal hot-top having a V-shaped crimp in its lower portion.

5. A sheet metal hot-top having a V-shaped crimp, and dimensioned for frictional engagement with the sides of the 80 mold.

6. A sheet metal hot-top crimped peripherally for increasing the facility of rupture of a casting at said crimp.

7. A sheet metal hot-top having a per- 85 ripheral, continuous, inwardly directed crimp.

8. A sheet metal hot-top having a peripher- 90 al, inwardly directed crimp, said hot-top having overlapping edges secured together and dimensioned for frictional contact with the interior of a mold.

9. A sheet metal hot-top having a continuous, peripheral, inwardly directed crimp in its lower portion, the edges of said sheet 95 metal overlapping and the hot-top dimensioned for frictional contact with the interior of a mold.

10. A sheet metal hot-top peripherally crimped, the cross-section of said crimp hav- 100 ing substantially parallel portions connected by a V-shaped wall.

11. A sheet metal hot-top crimped inwardly, of substantially the same composition as the metal to be cast therethrough, 105 and dimensioned for frictional contact with a mold.

12. A sheet metal hot-top of the composition of the metal to be cast, having a continuous groove forming an inwardly directed, continuous peripheral crimp and dimensioned for vertically adjustable frictional contact with the interior of a mold. 110

13. An imperforate sheet metal hot-top for welding connection with a casting, the 115 composition of which is the same composition as that of the metal of the casting.

In testimony that I claim the foregoing as my invention, I have signed my name hereto.

LEWIS B. LINDEMUTH.